

## UNITED STATES PATENT OFFICE

2,132,456

## DYEING CELLULOSE ESTERS AND ETHERS

Harold Blackshaw and Maurice Arthur Thorold Rogers, Blackley, England, assignors to Imperial Chemical Industries Limited, a corporation of Great Britain

No Drawing. Application August 4, 1936, Serial No. 94,262. In Great Britain August 14, 1935

3 Claims. (Cl. 8—5)

The present invention relates to the dyeing of textile materials composed of cellulose esters and ethers by means of triazene compounds, characterized by the presence of the group  $-\text{N}=\text{N}-\text{N}-$ , both water soluble and water insoluble, in conjunction with suitable coupling components. The amines used for the preparation of the diazo compounds which enter into the formation of the aforesaid triazenes are free from 10 water-solubilizing groups and may be mono- or polynuclear.

We have found that triazene compounds, e. g. that prepared from diazotized 5-chloro-2-toluidine and diethanolamine, are taken up by fibre 15 composed of cellulose ester or ether and are hydrolyzed and developed on the fibre by treatment in a bath containing a coupling component (as for example 2:3-hydroxynaphthoic acid) and an acid (either mineral or organic, as for example, 20 acetic or formic or dilute hydrochloric acid). Alternatively the coupling component, (as for example 2:3-hydroxynaphthoic acid anilide) may be applied to the fibre simultaneously with the triazene compound, and the shade then developed 25 on the fibre by treatment with acid.

The invention, accordingly, has for an object the provision of novel means of producing fast shades on cellulose ethers and esters; a further object is the production by novel means on 30 cellulose esters and ethers of ice colours; a further object is the production on cellulose esters and ethers of ice colours without application to the fibre of diazotizing baths. Other objects will become apparent as the description proceeds.

Generally speaking those triazene compounds free from water solubilizing groups, e. g. those derived from diazo compounds usually employed in the production of ice colours and from secondary amines free from carboxylic or sulphonic 40 groups are preferred because they have the greatest affinity for cellulose esters and ethers and yield on development the deepest shades. Of the water soluble compounds containing carboxylic or sulphonic groups or both the affinity 45 appears to be dependent to some extent on the chemical constitution. Thus the triazenes derived from cyanamide or cyanamide carboxylic acid usually possess better affinity than corresponding triazene compounds derived for example from sarcosine, sulphonanthranilic acid, 50 pipercolinic acid and the like.

In carrying the invention into effect it is usually preferred to mix the triazene compounds with a suitable dispersing agent, as e. g. Turkey-red oil or a salt of the condensation product of naphthalene sulphonic acid and formaldehyde to secure their better distribution in and absorption 55 from the dye bath.

In that embodiment of the invention in which 60 a triazene compound and a coupling component

are applied simultaneously to the fibre and development effected by subsequent immersion in a bath containing only acid, it is necessary that the coupling component shall have affinity for the cellulose ester or ether. Hence those preferably used are such as contain no solubilizing groups such as sulphonic or carboxylic groups, for instance, the arylamides of 2:3-hydroxynaphthoic acid. If sulphonic groups are present they should preferably be in the form of sulphuric esters, as for instance sulphatoethyl-meta-toluidine.

Hitherto developed shades are acetyl cellulose artificial silk (which is the most widely used substance of those coming within the group of textile materials composed of cellulose esters and ethers) have been obtained by causing a diazotizable base to be absorbed by the fibre in one bath, diazotizing the base on the fibre in another bath, and finally, coupling the thus produced diazo compound with a suitable component in a third bath.

According to the present invention no more than two baths are necessary for the production of a developed dyeing, thus not only is a considerable economy in time and labour effected, but beyond this, by the elimination of a process, the liability to damage of the valuable artificial silk.

As examples of triazene compounds adapted for use according to the invention, we mention, for instance, diazoimino or diazoamino compounds, prepared from diethanolamine, the tetra- and hexaethoxyamines (which are obtained by condensing four or six molecular proportions respectively of ethylene oxide with one molecular proportion of 4-toluene-sulphonamide and hydrolyzing the condensation product thus obtained with aqueous sulphuric acid of 60% strength), 35 6 - methyl - 2:2:4 - trimethyltetrahydroquinoline, isoindoline, ethylamino-p-toluidine, methylamino-p-toluidine, methylamine-benzene-p-sulphonamide, methylamine-benzene-p-dimethylsulphonamide, methylamino-p-dimethylamino-aniline, p-ethyl-amino-benzamide, tetrahydrocarbazole 40 45



dihydrobenzcarbazole



2:3:5-trimethyl-indole, cyclohexylmethylamine, 55



50

55

60

dimethylamine, diethylamine, dipropylamine, methylhydroxyethylamine, ethylhydroxyethylamine, dicyclohexylamine, methylamino-tetrahydronaphthalene

5



10

pyrrolidine, methylglucamine, ethylglucamine, sarcosine, pipecolinic acid, piperazine acetic acid, the alkali salts of cyanamide or cyanamide carboxylic acid, sulfoanthranilic acid, aniline disulphonic acid, piperidine sulphonic acid, methyltaurine, hydroxyethyltaurine, dibenzylamine disulphonic acid, methylaniline-p-sulphonic acid, methyl-aniline-m-sulphonic acid, methylaniline-p-carboxylic acid, ethyl-p-toluidine-sulphonic acid, monoglycinated 4-sulfoanthranilic acid, di-glycolamino acid

25



30

2-amino-4-sulphobenzoic acid, 3-amino-5-sulphobenzoic acid, 3-amino-5-sulpho-4-hydrobenzoic acid, 2-amino-5-sulphobenzoic acid, 5-sulpho-4-methyl-3-aminobenzoic acid, 1-aminobenzene-3:5-dicarboxylic acid, 4-aminobenzene-1:2-dicarboxylic acid, 4-amino-2-sulpho-oxanilic acid, piperazine-acetic acid.

35

By way of illustration of bases from which diazo compounds suitable for the production of triazene compounds may be prepared we mention among others as suitable bases 4:5-dichloro-2-amino-methylbenzene, 3:6-dichloro-4-amino-methylbenzene, 6-nitro-4-methoxy-3-amino-methylbenzene, 6-benzoylamino-4-chloro-3-amino-methoxybenzene, 4:6-dichloro-2-amino-1-methylbenzene, 2:5-dichloroaniline, 5-nitro-o-toluidine, 4-amino-5-benzoylamino-m-xylene, N-p-amino-benzoyl-p-toluidine,  $\alpha$ -aminoanthraquinone,  $\alpha$ -naphthylamine, 4-aminoazobenzene, 4-amino-5-methoxy-2-ethoxy-2-methylazobenzene, 5-chloro-o-toluidine, 4-chloro-2-nitroaniline, 3-amino-carbazole, tolidine, 1-amino-4-benzoylamino-2:5-diethoxyaniline, o-chloroaniline, 4-chloro-5-nitro-o-anisidine, m-nitraniline, 4-chloro-o-anisidine, 6-chloro-o-toluidine, 2-benzoylamino-5-amino-cresol ether.

40

By way of illustration of coupling components which may be applied simultaneously with the triazene compound to the fibre or which may be added to the acid coupling bath we mention acetoacet-o-tolidide, acetoacet-p-chloraniline, the arylides of 2:3-hydroxynaphthoic acid, for instance, the anilide, 4-bromo-o-anilide, 2:5-dimethoxyanilide,  $\alpha$ -naphthylamide, diaminide, m-nitranilide, p-chloranilide, 5-methoxy-2-toluidide, o-anisidine, p-anisidine,  $\beta$ -naphthylamide, 5-chloro-2-toluidide, o-phenetidine, m-xylidine, p-chloroanilide of 2-hydroxy carbazole-3-carboxylic acid, o-toluidide of 2-hydroxyanthracene-3-carboxylic acid, resorcinol, m-phenylene diamine, 4-hydroxydiphenyl-3-carboxylic amide, 3-hydroxydiphenylamine-5-carboxylic amide, 3-hydroxydiphenylamine-4-carboxylic amide, 3-hydroxydiphenylether-5-carboxylic amide, 2:4-dihydroxyquinoline, 2:4-hydroxybenzquinoline, 1-hydroxy-naphthyl 4-phenylketone, 1:5-hydroxynaphthol, 1:5- $\beta$ -hydroxyethylaminonaphthol, 6-chloro-2:3-hydroxynaphthoic amide, 6-ethoxy-2:3-hydroxynaphthoic anilide, 2:6-dihydroxynaphthalene-3:7-dicarboxylic anilide, 3:6-

dihydroxynaphthalene-2:6-dicarboxylic anilide, hydroxyphenanthrene-o-carboxylic anilides, hydroxychrysene-o-carboxylic anilides, arylalkylpyrazolones, e. g. phenylmethylpyrazolone,  $\alpha$ -naphthol,  $\beta$ -naphthol, aminonaphthols, 3-hydroxycarbazole, 3-hydroxyfluorene, 3-hydroxyfluorene-2-carboxylic-o-toluidide, 3-hydroxy-diphenylene oxide, 3-hydroxy-diphenylene oxide-2-carboxylic-p-chloranilide, 1:5-(hydroxyethylamino)-naphthol, hydroxyanthracenes, hydroxyphenanthrenes, but it is to be understood that other suitable coupling components may be employed.

As examples of cellulose esters and ethers to which the process of the invention may be applied we mention acetyl, formyl, propionyl and butyryl cellulose, benzyl, methyl, ethyl, propyl and butyl cellulose.

The following examples illustrate but do not limit the invention. The parts are by weight.

#### Example 1

The triazene compound used in this example is made as follows:—

7 parts of p(p'-aminophenylazo)- $\alpha$ -naphthylamine are dissolved in 50 parts of water and 11 parts of hydrochloric acid, sp. gr. 1.16, cooled to 0° C. and treated with 25 parts of sodium nitrite solution (14%). The solution thus obtained is run into a solution containing 7 parts of secondary hexaethoxyamine (prepared by condensing six molecular proportions of ethylene oxide with 1 molecular proportion of 4-toluenesulphonamide and hydrolyzing the resultant product with 60% sulphuric acid) and a large excess of sodium carbonate. The black precipitate which is formed is filtered off and ball-milled with 25% of its weight calculated as dry compound, of the sodium salt of the condensation product of naphthalene sulphonic acid and formaldehyde and 10% water.

A bath is made up from 32 parts of this mixture, 2 parts of soda ash and 3000 parts of water. Into this bath at ordinary temperature there is introduced 100 parts of acetate rayon. The temperature is gradually raised to 50° C., which is maintained for  $\frac{1}{4}$  hour.

The colour is developed in a bath consisting of 3000 parts of water, 5 parts of  $\beta$ -hydroxynaphthoic acid (liberated from its sodium salt by acetic acid) and 10 parts of acetic acid (30%) at 85° C. for  $\frac{1}{2}$  hour. The material is then washed and dried. A black shade is obtained.

#### Example 2

The triazene compound used in this example is prepared as follows:—

7.6 parts of aminoazotoluene are diazotized by stirring for  $\frac{1}{2}$  hour with 11.1 parts of hydrochloric acid (sp. gr. 1.16), 50 parts of water and 25 parts of sodium nitrite solution (14%); the aqueous solution is then filtered and run slowly with agitation into a solution containing 14 parts of secondary hexaethoxyamine prepared as aforesaid and an excess of sodium carbonate; a thick dark coloured oil separates, which readily gives a clear solution in water in the presence of one of the usual dispersing agents, such as Turkey-red oil.

Acetate rayon is dyed a bright yellow by means of the above triazene in the manner described in Example 1. The shade rapidly develops in a bath of beta-hydroxynaphthoic acid made acid with acetic acid and heated to 80° C. to violet or purple shades.

**Example 3**

The triazene compound used in this example is prepared as follows:—

5 93 parts of aniline are diazotized and slowly added to 85 parts of piperidine in 200 parts of water and an excess of sodium carbonate with stirring. The oil which is formed is removed by extraction with ether and the ether evaporated off. The oily diazoimino compound is mixed intimately with 20% by weight of Turkey-red oil (50% soda finished). The resultant paste readily disperses in hot water (80° C.).

10 15 Acetate rayon is dyed a dull yellow with the above compound as described in Example 1. Development is effected by treatment with a hot (80° C.) solution of the sodium salt of 2:3-hydroxynaphthoic acid acidified with acetic acid. A brilliant scarlet shade is obtained.

**Example 4**

20 25 3.5 parts of the re-dispersible diazoimino preparation, made as described in Example 8 are pasted with 1.75 parts of Turkey-red oil (50% soda finished) and added to the dye vessel which contains 5 parts of trisodium phosphate, 20 parts of common salt and 3000 parts of water. 100 parts of acetate rayon is worked in this bath as described in Examples 8, 9 and 10.

30 35 The treated material is developed in a bath at 80° C. containing 6 parts of acetic acid (50% aqueous solution), 6 parts of a 25% paste of sodium N-oleyl-4-amino-1-methoxy-benzene-2-sulphonate, and 3000 parts of water, to which has been added 2 parts of the anilide of 2:3-hydroxynaphthoic acid mixed with 7.5 parts of a 10% glue solution.

40 Development is complete in half an hour, and the dyeing is then rinsed well. A bright scarlet shade is obtained.

**Example 5**

A triazene compound is prepared as follows:—  
6.3 parts of the azo dyestuff



50 55 are stirred at room temperature with 100 parts of water and 14 parts of 10 N hydrochloric acid. There is run in, over a period of half an hour, 3.45 parts of sodium nitrite dissolved in 25 parts of water. The solution is stirred a further 1/2 hour, filtered, and run slowly into 6 parts of diethanolamine dissolved in 100 parts of 2N. sodium carbonate solution. The reddish coloured precipitate is filtered, washed, ball milled with 50 parts of a 50% solution of the sodium salt of the condensation product of naphthalene sulphonic acid and formaldehyde and the resulting paste dried and ground thoroughly.

60 65 2.1 parts of the above ground powder are stirred into a dyebath containing water (5000 parts) and soda ash (2 parts), 100 parts of acetate rayon entered, worked for 1 hour at a temperature of 80-85° C., then rinsed in cold water and developed for half an hour in a bath containing 5000 parts of water, 5 parts of 2:3-hydroxynaphthoic acid and 10 parts of acetic acid (30%) for 1/2 hour.

70 A bright blue shade is obtained.

**Example 6**

A bath is prepared containing 10% on the 75 weight of material to be treated of an equimo-

lecular mixture of the diazoimino compound prepared from diazotized 5-chloro-o-toluidine and secondary hexaethenoxyamine, prepared as described in Example 1, and the sodium salt of 2:3-hydroxynaphthoic anilide. Acetate rayon is 5 treated in this bath at 80° C. for 10 minutes. It takes up both compounds. The almost colourless material is lightly rinsed with water and developed by immersion for half an hour at 80° C. in a bath containing 10% of acetic acid 30% 10 (calculated on the weight of material). A brilliant red shade is obtained.

**Example 7**

15 In 1000 parts of a dyebath containing 1.25 parts of the diazoimino compound of p(p'-aminophenylazo)- $\alpha$ -naphthylamine and secondary hexaethenoxyamine, prepared as described in Example 1, and 1 part of the sodium salt of sulphonatoethyl-meta-toluidine, acetate rayon (25 20 parts) is introduced and manipulated as previously described. When immersed in a bath at 80° C., containing 10% acetic acid (30%) (calculated on the weight of material), a deep reddish-brown is developed. 25

**Example 8**

A triazene compound is prepared as follows:—  
282 parts of 5-chloro-2-toluidine are diazotized 30 in the usual manner, and the diazo solution is run slowly into a well stirred solution of 172 parts of diethanolamine in 2500 parts of water, made alkaline by the addition of 500 parts of soda ash. The addition of some solid condensation product from a previous preparation before addition of the diazo solution is advisable to prevent the diazoimino compound separating out as an oil which may take some time to solidify.

The thus obtained solid product is filtered and 40 washed with cold water. The paste is mixed with 1500 parts of a 50% aqueous solution of the sodium salt of the condensation product of naphthalene sulphonic acid and formaldehyde, and ball-milled for two hours. The paste so obtained 45 is dried at 50° C. and ground to a very fine powder.

Such a powder disperses readily in cold water and dissolves to a clear solution in warm water. 50 55 3.5 parts of the above powder is pasted with 1.75 parts of Turkey-red oil (50% soda finished) and 35 parts of water at a temperature of 60° C. added. 2.0 parts of the 5-chloro-2-toluidide of 2:3-hydroxynaphthoic acid are pasted with 0.33 parts of the sodium salt of the acid sulphuric ester of the alcohols obtained by the saponification of sperm oil and diluted with 20 parts of water at a temperature of 40° C. The above are added to the bath which contains 6 parts of trisodium phosphate, 10 parts of sodium chloride and 3000 parts of water at a temperature of 40° C. 60 65 100 parts of acetate rayon yarn are entered and worked for 1/4 hour during which time the temperature of the bath is raised to 80° C. and dyeing continued for 3/4 hour. The almost colourless material is then well rinsed in cold water and treated in a bath at 80° C. prepared by the addition of 60 parts of acetic acid (50%) to 3000 parts of water, worked for 1/2 hour at this temperature and well rinsed in cold or warm (40° C.) water. It is then soaped in a bath containing 3 70 75 parts of soap flakes per 1000 parts of water.

If the acetate rayon is lustrous, it is worked at a temperature of 80° C. for 1/2 hour. If delustered material is used, the temperature may be raised to 95-98° C. 76

A bright bluish-red shade is obtained of very good fastness to washing.

*Example 9*

5 A triazene compound is prepared as follows:—  
 30 parts of 4-benzoylamino-2:3-diethoxyaniline are added slowly to a boiling mixture of 300 parts of water and 12 parts of 10 N hydrochloric acid, and boiling is continued until a clear solution is obtained. This solution is cooled to 5° C. with stirring, a further 16 parts of 10 N hydrochloric acid added and the suspension diazotized with a saturated solution containing 6.9 parts of sodium nitrite. The filtered diazo solution is run slowly into 11.5 parts of diethanolamine dissolved in 150 parts of 2N-sodium carbonate solution, which is seeded during the early part of the addition with solid product obtained from a previous preparation. A brown granular precipitate is obtained which is filtered from the liquor, washed with cold water, and ball-milled for 3 hours with 40 parts of the condensation product of sodium naphthalene sulphonate and formaldehyde, 100 parts of water and 20 parts of a 25% paste of sodium N-oleyl-4-amino-1-methoxybenzene-2-sulphonate. The product is dried at 50° C. and ground, giving a readily dispersible powder.

3.5 parts of the above powder are pasted with 1.75 parts of Turkey-red oil (50% soda finished). The paste is diluted with 35 parts of water at a temperature of 60° C. Further, 1.0 part of the

development performed as described in Example 8. A bright greenish-blue shade of good fastness properties is obtained.

*Example 10*

A triazene compound is prepared as follows:—  
 3.5 parts of the diazoimino compound prepared from diazotized 2:5-dichloroaniline and cyanamide carboxylic acid by running the diazo solution into an equimolecular amount of cyanamide dissolved in water and maintaining alkaline throughout by the addition of sodium bicarbonate, are pasted with 1.75 parts of Turkey-red oil (50% soda finished) and diluted with 35 parts of water at a temperature of 60° C.

5.0 parts of 5-chloro-2-toluidide of 2:3-hydroxynaphthoic acid are pasted with 2.5 parts of a 33% aqueous paste of the sodium salt of the acid sulphuric ester of the alcohols obtained by the sulphonation of sperm oil, and diluted with 50 parts of water at a temperature of 60° C. and, together with the dispersed diazoimino compound, added to the dye vessel which contains 6 parts of trisodium phosphate, 30 parts of sodium chloride and 3000 parts of water at a temperature of 40° C.

Dyeing and further procedure may be carried out as described in Example 8.

An orange shade of good fastness is obtained.

The following table illustrates further combinations and shades obtained therefrom when applied according to the invention.

| No. | Diazotized base                                                                                                                                                                                                                                                                    | Combined with—                                                                                                                                                                                      | Coupling component                                        | Shade                      |
|-----|------------------------------------------------------------------------------------------------------------------------------------------------------------------------------------------------------------------------------------------------------------------------------------|-----------------------------------------------------------------------------------------------------------------------------------------------------------------------------------------------------|-----------------------------------------------------------|----------------------------|
| 35  | 1. 5-chloro-2-toluidine                                                                                                                                                                                                                                                            | Diethanolamine                                                                                                                                                                                      | 4:4'-diacetacet-2-toluidide                               | Bright greenish yellow. 35 |
|     | 2. do                                                                                                                                                                                                                                                                              | CH <sub>2</sub> CH <sub>2</sub> OCH <sub>2</sub> CH <sub>2</sub> OH                                                                                                                                 | 4-chloroanilide of 2-hydroxy-carbazole-3-carboxylic acid  | Deep brown.                |
|     | 3. 4-benzoylamino-2:5-diethoxyaniline.                                                                                                                                                                                                                                             | Diethanolamine                                                                                                                                                                                      | 2-toluidide of 2-hydroxyanthracene - 3 - carboxylic acid. | Bright bluish green.       |
| 40  | 4. do                                                                                                                                                                                                                                                                              | Morpholine                                                                                                                                                                                          | Anilide of 2:3 hydroxynaphthoic acid.                     | Blue.                      |
| 40  | 5. Aniline                                                                                                                                                                                                                                                                         | Diethanolamine                                                                                                                                                                                      | do                                                        | Scarlet. 40                |
|     | 6. 5-chloro-2-toluidine                                                                                                                                                                                                                                                            | do                                                                                                                                                                                                  | 2-naphthol                                                | Bright reddish orange.     |
|     | 7. 6-chloro-2-toluidine                                                                                                                                                                                                                                                            | do                                                                                                                                                                                                  | 3-nitroanilide of 2:3-hydroxynaphthoic acid.              | Yellowish red.             |
| 45  | 8. o-Aminoazo-toluene                                                                                                                                                                                                                                                              | Secondary hexaethoxy-amine.                                                                                                                                                                         | 4-chloroanilide of 2-hydroxy-carbazole-3-carboxylic acid  | Deep brown.                |
|     | 9. 3-chloroaniline                                                                                                                                                                                                                                                                 | Secondary tetraethoxy-amine.                                                                                                                                                                        | 5-chloro-2-toluidide of 2:3-hydroxynaphthoic acid.        | Yellowish scarlet.         |
|     | 10. 4-chloro-2-toluidine                                                                                                                                                                                                                                                           | Diethanolamine                                                                                                                                                                                      | 3-nitroanilide of 2:3-hydroxynaphthoic acid.              | 45                         |
| 50  | 11. 4-nitro-2-aminoanisole.                                                                                                                                                                                                                                                        | do                                                                                                                                                                                                  | do                                                        | Bright bluish-red.         |
|     | 12. 4-benzoylamino-2:5-diethoxyaniline.                                                                                                                                                                                                                                            | do                                                                                                                                                                                                  | Anilide of 2:3-hydroxynaphthoic acid.                     | Bright reddish-blue.       |
|     | 13. Dianisidine                                                                                                                                                                                                                                                                    | do                                                                                                                                                                                                  | 4:4'-diacetacet-2-toluidide                               | Deep gold.                 |
| 55  | 14. $\alpha$ -naphthylamine                                                                                                                                                                                                                                                        | do                                                                                                                                                                                                  | 3-nitroanilide of 2:3-hydroxynaphthoic acid.              | Light bordeaux. 50         |
|     | 15. 3 - benzoylamino - 4 - methoxyaniline.                                                                                                                                                                                                                                         | do                                                                                                                                                                                                  | 5 - chloro - 2 - toluidide of 2:3-hydroxynaphthoic acid.  | Bright reddish blue.       |
|     | 16. 5-chloro-2-toluidine                                                                                                                                                                                                                                                           | N - carbethoxypiperazine                                                                                                                                                                            | do                                                        | Do.                        |
| 55  | 17. 1 - amino - anthraquinone.                                                                                                                                                                                                                                                     | Diethanolamine                                                                                                                                                                                      | Anilide of 2:3-hydroxynaphthoic acid.                     | Bright red.                |
|     | 18. 2 - benzoylamino - 4 - chloro - 5 - aminoanisole.                                                                                                                                                                                                                              | do                                                                                                                                                                                                  | 2-anisidide of 2:3-hydroxynaphthoic acid.                 | Rich violet. 55            |
|     | 19. do                                                                                                                                                                                                                                                                             | do                                                                                                                                                                                                  | 5 - methoxy - 2 - toluidide of 2:3-hydroxynaphthoic acid. | Violet.                    |
| 60  | 20. 2:5-dichloroaniline                                                                                                                                                                                                                                                            | Cyanamide                                                                                                                                                                                           | 5-chloro-2-toluidide of 2:3-hydroxynaphthoic acid.        | Orange.                    |
|     | 21. Anisole                                                                                                                                                                                                                                                                        | do                                                                                                                                                                                                  | 4-bromo-2-anisidide of 2:3-hydroxynaphthoic acid.         | Dull yellowish red. 60     |
|     | 22. 4-chloro-2-nitroaniline                                                                                                                                                                                                                                                        | do                                                                                                                                                                                                  | 3-nitroanilide of 2:3-hydroxynaphthoic acid.              | Red.                       |
| 65  | 23. 5-nitro-2-aminoanisole.                                                                                                                                                                                                                                                        | N - ethylaniline - 4 - sulphonnic acid.                                                                                                                                                             | do                                                        | Dull red.                  |
|     | anilide of 2:3-hydroxynaphthoic acid                                                                                                                                                                                                                                               | are pasted with 0.15 part of the sodium salt of the acid sulphuric ester of the alcohols obtained by the saponification of sperm oil, and diluted with 10 parts of water at a temperature of 60° C. |                                                           |                            |
| 70  | The above dispersed diazoimino compound and coupling component are added to the dye vessel which contains 2.4 parts of soda ash, 10 parts of sodium chloride and 3000 parts of water at a temperature of 40° C. 100 parts of acetate rayon yarn are entered and the dyeing and de- |                                                                                                                                                                                                     |                                                           |                            |

The amino derivative used in the second column of the second example in the table is prepared by reacting N-ethyl- $\alpha$ -naphthylamine or N-ethylaniline with 2 molecular proportions of ethylene oxide, converting into the 4-nitroso compound with nitrous acid, and hydrolyzing with hot aqueous caustic soda.

We claim:

1. A process of dyeing cellulose ester and ether materials which comprises applying to the material a bath containing a triazene compound 75

5 prepared from a diazotized aryl amine which upon acidification yields a diazo salt that is capable of coupling with an azo dye coupling component, said bath being alkaline and containing sufficient base to prevent the splitting-off of a diazo salt from the triazene compound but an insufficient quantity and concentration of base to saponify said material, and then developing in the presence of an azo dye coupling component by applying an acid bath.

10 2. The process of dyeing cellulose ester and ether material which comprises applying to the material a bath containing a triazene compound prepared from a diazotized arylamine which upon acidification yields a diazo salt, said bath being alkaline and containing sufficient base to prevent the splitting-off of a diazo salt from the triazene compound but an insufficient quantity and concentration of base to saponify cellulose ester and ether materials, and then developing by applying an acid bath of an azo dye coupling component.

15 3. In the process of dyeing in which a com-

pound capable of coupling with a diazo compound and a triazene compound prepared from a diazotized primary aryl amine which is capable of yielding a diazo salt upon acidification are applied to cellulose ester and ether materials 5 which are to be dyed and the dye is developed by acidification, the steps which comprise first immersing said material in an alkaline dyeing medium comprising the triazene compound, a coupling component having affinity for said material, a dispersing agent and a solution of a base which contains an insufficient quantity and concentration of the base to saponify the cellulose ester and ether material and to convert the coupling component to its alkali metal salt but sufficient base to prevent the regeneration of a diazo salt from the triazene compound, and thereafter developing by applying a solution containing an acid which is effective to regenerate a diazo salt 10 from the triazene compound. 15 20

HAROLD BLACKSHAW.

MAURICE ARTHUR THOROLD ROGERS.